

A. E. WHEELER & M. W. KREJČI.  
PROCESS OF FORMING FURNACE LININGS.  
APPLICATION FILED DEC. 4, 1912.

1,068,470.

Patented July 29, 1913.



WITNESSES:

Harry A. Beinez  
Rannie C. Weber.

INVENTORS.  
Archer E. Wheeler and  
Milo W. Krejči.  
BY *Emile Starek*  
ATTORNEY.

# UNITED STATES PATENT OFFICE.

ARCHER E. WHEELER AND MILO W. KREJČI, OF GREAT FALLS, MONTANA.

## PROCESS OF FORMING FURNACE-LININGS.

1,068,470.

Specification of Letters Patent Patented July 29, 1913.

Application filed December 4, 1912. Serial No. 734,889.

*To all whom it may concern:*

Be it known that we, ARCHER E. WHEELER and MILO W. KREJČI, citizens of the United States, residing at Great Falls, in the county of Cascade and State of Montana, have invented certain new and useful Improvements in Processes of Forming Furnace-Linings, of which the following is a full, clear, and exact description, reference 10 being had to the accompanying drawings, forming a part hereof.

Our invention has relation to improvements in processes of forming furnace linings, and it consists in the novel features 15 more fully set forth in the specification, and pointed out in the claims.

In the drawings, the figure represents a vertical middle section of a copper converter showing our invention applied 20 thereto.

The present invention though here shown as directed to the protection of the basic lining of a copper converter, generically contemplates the protection of the linings 25 of any metallurgic or smelting furnace, crucible, or other vessel, the object of the invention being to form *in situ*, or directly on such lining, as a foundation, a protecting coat which will protect such foundation 30 against the corrosive action of the charge normally treated in said furnace. In the example here selected, we apply our invention to the basic lining of a copper converter, such lining being usually composed 35 of magnesite brick, (or other equivalent material,) the said lining serving as a foundation to which our protecting layer may adhere. It is to be understood, however, that we do not wish to restrict the application 40 of our invention to protecting layers for basic linings, but desire to apply the layer to any foundation whatsoever to which the layer will adhere.

A further object is to provide a protecting 45 layer which is practically infusible, or fusible with difficulty at the prevailing temperatures at which the usual furnace-charge is treated, the composition of the layer being such as not to enter into chemical combination either with any of the elements of the charge while the latter is being treated, or with the foundation which the layer is designed to protect. The inert, and relatively infusible character of the protecting layer,

by virtue of its lasting qualities, dispenses 55 with the frequent renewals and repairs of furnace and converter linings, now so generally necessary where smelting and refining operations are carried on. By our invention the protecting layer is directly derived 60 and segregated from, the charge introduced into the furnace, the segregating process resulting from the oxidation (or conversion into infusible compounds) of certain metallic bases (present in the charge) 65 without the addition of fluxes, all as will be more fully apparent from a detailed description of the invention, which, when applied to a basic lined copper converter, may be described as follows:

Referring to the drawings, C represents the outer shell of an "upright" type of converter, W the wind-box, T the tuyers, and M the basic lining thereof, in the present case composed of magnesite brick, all as well 70 understood in the art. No means for tipping or tilting the converter are here shown as they constitute no part of the present invention; besides any means known to the art may be improvised, it being sufficient 75 for our present purpose to bear in mind that the converter is tiltable as is usual with this type of furnace.

The protecting layer forming the subject-matter of the present improvement is represented by the reference symbol L, said layer ranging anywhere from two to six inches in thickness. This layer is derived directly from a charge of matte blown in the converter, the charge averaging about 80 eighteen inches in depth above the center line of the tuyers, the level of said charge being indicated by the dotted line x. Matte, as is well known is a sulfid of copper (Cu<sub>2</sub>S) containing an admixture of sulfid 85 of iron (FeS) and other impurities. When a charge of matte is blown in a converter provided with a basic lining, a silicious flux is added in the shape of silica or silicious ore, the same forming a silicate or slag with 90 the iron (and other bases constituting the impurities), the sulfur of the iron (and any free sulfur if present) being first oxidized to SO<sub>2</sub>, which passes off as a gas and the iron being converted into a ferrous oxid 95 readily combinable with the added fluxes. The slag floating on top of the charge is 100 removed, leaving Cu<sub>2</sub>S or "white metal" 105

in the converter, which upon further blowing is converted into metallic copper, the reaction being substantially as follows:—



that is to say, a portion of the copper sulfid is first oxidized to the first oxid, which in turn reacting with unconverted portions of 10 the sulfid reduces the latter, the sulfur being oxidized to  $\text{SO}_2$ .

The foregoing reactions substantially represent the steps of conversion from matte to metallic copper and are here outlined to better illustrate the application of our invention. This contemplates the blowing of an initial charge of matte without the addition of fluxes (silica or silicious ore) the oxygen infused or introduced into the 20 charge by the blast oxidizing the iron (the sulfur being converted into  $\text{SO}_2$  gas) without disturbing the copper sulfid, sulfur, as is well understood having greater affinity for copper than for iron. The iron oxids 25 thus formed not being susceptible of combination with the basic lining of the converter, and being left free and non-combined with any suitable flux, segregate themselves from the copper sulfid (white metal) and 30 adhere more or less to the magnesite lining. In the practical operation of our process the charge is blown (without flux) for a short time to a temperature not in excess of 2600 degrees Fahrenheit, the blast being then cut 35 off and the converter turned down to cool, in which turning down the material runs over the magnesite foundation M, a layer of the segregated iron oxids adhering thereto along such portions as it will. The converter is then turned up again and blown 40 for a short period (without flux) and again turned down and allowed to cool (say from ten to twenty minutes) when the iron oxids will adhere to other portions of the basic 45 lining. Considerable portions of the layer of iron oxids are of course distributed over the magnesite foundation by the splashing of the contents during the blowing, and these added to the portions adhering to such 50 foundation each time the converter is turned down, form an aggregate protecting layer of the desirable thickness in the majority of cases. Where the quantity of iron in an initial charge of matte (the charge being usually from twelve to eighteen inches above 55 the tuyers) is insufficient to furnish the necessary quantity of iron oxids for a desired thickness of the protecting layer, the copper sulfid or white metal remaining upon 60 the exhaustion of the iron, is removed from the converter, and another charge of matte is added and blown (without flux) and the operations are repeated until a layer of proper thickness has accumulated. This 65 layer as previously stated, may be from two

to six inches in thickness. Where matte is the charge initially blown, the segregated oxid is decidedly magnetic and is probably a mixture of  $\text{Fe}_2\text{O}_3$  and  $\text{Fe}_3\text{O}_4$ , though its precise composition is not here attempted to be defined. At the temperature at which matte is blown for copper conversion (when flux is added to the charge to slag the iron) the layer of iron oxids above described, is practically infusible or fusible with difficulty, so that in the normal operations of the converter the layer of oxid protects its basic foundation for a considerable period of time, thus prolonging the life of the converter. When flux (silica or silicious ore) is 70 added to the charge in the normal operation of copper conversion, the heat generated by the blast and oxidation of the iron is absorbed in the melting of the flux so that the temperature of copper conversion is always considerably lower than that to which the initial charge was raised during the formation of the layer of iron oxids or protecting coating. In forming the coating the temperature in fact rises very rapidly and that is 75 the reason why the charge is left to cool and the converter turned down, an excessive heat not only being destructive to the vessel but retarding in a measure the desired segregation of the iron oxids from the white metal 80 or copper sulfid. Where subsequent charges of matte are regularly blown in a converter whose lining is protected by a layer such as 85 here described, the layer is practically inert or infusible because the temperatures at 90 which the normal operations are carried on never rise high enough to attack the protecting layer. In the regular or normal blowing of copper, the flux added to the charge combines with the iron so that it 95 leaves the protecting layer intact, and the temperature of conversion being below the fusing point of the layer, the latter is not disturbed. Of course, in practice the coat 100 of oxid will vary or fluctuate in thickness, 105 sometimes becoming thinner and at times increasing in thickness. When it becomes too thin a charge may be blown with a deficiency of flux, which would have the effect of depositing oxid on the layer and thus increasing 110 its thickness; if the layer became too thick, a charge may be blown at an increased temperature which will reduce the thickness, or an excess of flux may be added 115 which will slag off a part of the coat, or both high temperature and an excess of flux 120 may be resorted to.

It is of course, to be understood that the foundation for the inner protecting layer or coat need not be a basic one, the magnesite 125 lining M being here selected merely by way of example; neither is it to be understood that we are to be restricted to a method of forming the coat without the use of a flux, because in some particular applications of 30

our process it might be desirable to add flux for the purpose of forming some particular compound; neither are we to be limited to the formation of iron oxids, because any 5 equivalent thereof segregated from an initial charge, and whose fusing point is above the temperature at which the charge is to be worked in the vessel afterward, is contemplated by our invention, provided the coat is formed in place or *in situ* from the molten contents of the vessel. For example, if some compound of aluminum were fused in a vessel and subsequently blown, the aluminum oxid  $Al_2O_3$  thus formed and adhering to the 10 inner walls of the vessel would be an equivalent of the iron oxids described above. For convenience it may be well to designate the protecting coat or layer L as a lining, and the magnesite layer M as the foundation, it 15 being understood that we do not limit ourselves to any particular kind of foundation nor to any specific composition of lining, those here described serving as convenient examples where our invention is applied to 20 coating the insides of copper converters lined with magnesite.

It may be stated in passing that when a newly lined converter is put into action after having been first properly heated, it has 25 been the usual practice to first treat one or more charges of "white metal" ( $Cu_2S$ ) so as to coat the lining (foundation), or to first treat one or more charges of matte to which charge or charges a flux containing 30 silica in some form is added, and allow, or deliberately attempt to make, the material coat over the lining of the converter. Such a coat however, when successfully formed, is merely a portion of the charge treated, and 35 is not formed or segregated from, the charge as an independent, inert, infusible layer or compound such as contemplated by our process. A coat resulting from the adhesion of a portion of the treated charge of white 40 metal, or a charge of matte to which flux has been added is short-lived, and being composed in the main of  $Cu_2S$  is reduced to metallic copper by reacting with the copper 45 oxid formed in the blowing of a regular charge as already pointed out in the re- 50 action in connection with copper conversion. Under our process, what adheres to the foundation is an inert layer segregated from the charge, such layer being practically a 55 unitary or monolithic infusible coat or sheet spread over the inner walls of the converter. Its inertness is due to the fact that it does not combine with the regular charges nor- 60 mally treated in the converter, the iron and other impurities in said charges being slagged off by a proper complement of added fluxes, the thickness of the coat being controlled by a proper regulation of the fluxes so added, and by the temperature of 65 the blow as already outlined. The generic

principle of our invention is the segregation of a component part of a molten charge and the conversion of such component into an inert, infusible compound which will adhere to the walls of the furnace or converter, the 70 conversion being preferably brought about by the oxidation of the metallic base of said component. The invention is further characterized by the fact that the segregated compound forms a coat or lining *in situ*, or 75 directly on the furnace wall from the molten charge treated in the furnace. By thus blowing a charge of matte in a newly lined converter without the addition of flux, and causing the segregated iron oxids to be 80 spread over the lining by the conjoint action of the blast and by properly tilting, or turning down of the converter, an inert, in- 85 tegral, infusible coat will be formed which will protect the original lining or founda- 90 tion for an indefinite period of time during the subsequent normal operations of the con- 95 verter. Should the protecting coat become detached for any reason, it may be readily renewed by blowing a charge without flux or 100 with a deficiency of flux, as will appeal to 105 the skilled operator.

The process herein may be practised not only in the treatment or conversion of cop- 95 per, but is equally applicable in the treat- 100 ment or converting of nickel, copper-nickel, iron, steel, and other metals; neither is it to be restricted in its application to converters, but may be practised with other forms of smelting, reducing, or metallurgical fur- 105 naces, be the same movable or stationary. To avoid a wasting away of the protecting coat or lining, care should be exercised in the normal operation of the converter to keep down the quantity of flux to a point where it 110 will no more than satisfy the iron of the matte constituting the charge being blown, otherwise any excess of flux (silica) will slag the lining and in time destroy it, there- 115 by necessitating frequent renewals. This matter however, will be understood by the operator and no such consequences need arise.

Having described our invention, what we 115 claim is:

1. In the formation of furnace linings, the process of introducing a molten charge into the furnace, diffusing oxygen through the charge and thereby segregating there- 120 from *in situ* a free oxidized compound ad- herable to the furnace walls and forming a lining therefor.

2. In the formation of furnace linings, the process of fusing a charge within the fur- 125 nace, introducing from without a current of oxygen into the charge, thereby segregat- ing from the charge *in situ* a component convertible into a free oxidized compound infusible at the temperature of normal operation of the furnace, and causing said 130

compound to adhere to the inner walls of the furnace and form a lining therefor.

3. In the formation of furnace linings, the process of delivering an oxidizing agent to a fused composite metallic charge thereby oxidizing suitable base components of said charge, segregating *in situ* the oxids of the base metals thus formed, and causing a diffusion thereof over the inner surface of the furnace.

4. In the formation of converter linings, the process of delivering currents of air to a fused composite metallic charge thereby oxidizing suitable base components of said charge, segregating *in situ* the oxids of the base metals thus formed, and causing a diffusion thereof over the inner surface of the converter.

5. In the formation of converter linings, the process of delivering currents of air to a fused composite metallic charge thereby oxidizing suitable base components of said charge, segregating *in situ* the oxids of the base metals thus formed, and causing a diffusion thereof in sheet form over the inner surface of the converter.

6. In the formation of copper converter linings, the process of blowing a charge of matte in a converter provided with an inner basic layer, oxidizing the iron and sulfur of the charge without the addition of flux and thereby segregating the oxids of the base metal thus formed, diffusing said segregated oxids over the surface of the basic layer whereby an inert, infusible, monolithic layer of iron oxids is formed on the basic layer.

7. In the formation of converter linings, the process of blowing a charge of matte in a converter provided with an inner layer serving as a foundation, oxidizing the metals of the compounds forming the impurities of the matte without the presence of fluxes, whereby the oxids of the base metals become segregated from the copper to be recovered, and manipulating the converter to cause the segregated oxids to distribute themselves as a sheet over the foundation layer.

8. In the formation of furnace linings, the process of fusing a charge containing a mixture of metallic compounds a portion of whose oxidized bases fuse at a higher tem-

perature than the oxids of the metals to be recovered, introducing oxygen and thereby oxidizing the metals whose oxids have the higher fusing point, *in situ*, whereby the same becomes segregated from the compounds of the metals to be recovered, and causing a diffusion of the oxids so formed over the inner surface of the furnace whereby an inert, infusible, monolithic coat or layer is formed.

9. In the formation of furnace linings, the process of fusing a charge composed of a mixture of metallic sulfids the sulfur of which has greater affinity for a portion of the metals than for the remaining portion, blowing the charge without the presence of fluxes to oxidize the sulfur and the metals for which the sulfur has the least affinity, and segregating *in situ* the oxids of said last mentioned metals, and causing a diffusion of said oxids over the inner surface of the furnace whereby an inert, infusible monolithic layer is formed capable of resisting the temperature resulting from the blowing of subsequent charges in the presence of fluxes.

10. In the formation of converter linings, the process of blowing a composite metallic charge and oxidizing suitable base components thereof without the addition of fluxes, segregating *in situ* the oxids of the base metals thus formed and causing a diffusion of the same in sheet form over the inner surface of the converter.

11. In the formation of furnace linings, the process of fusing a charge composed of compounds of mixed bases, infusing into the charge a complement of oxygen sufficient to oxidize a portion of said bases, whereby the same becomes segregated *in situ*, and causing a diffusion of said segregated oxids in sheet form over the inner surface of the furnace.

In testimony whereof, we affix our signatures in presence of two witnesses.

ARCHER E. WHEELER.  
MILo W. KREJCI.

Witnesses:

C. R. KUZELL,  
T. P. CORCORAN.